

# UNITED STATES PATENT OFFICE.

HENRY PEMBERTON, OF EAST TARENTUM, PENNSYLVANIA.

## IMPROVEMENT IN THE MANUFACTURE OF PAPER FROM SORGHUM.

Specification forming part of Letters Patent No. 38,059, dated March 31, 1863; antedated October 1, 1862.

*To all whom it may concern:*

Be it known that I, HENRY PEMBERTON, of East Tarentum, in the county of Allegheny and State of Pennsylvania, have invented a new and useful Improvement in the Manufacture of Paper; and I do hereby declare the following to be a full, clear, and exact description thereof.

The article which I use as a substitute for linen and cotton rags in the manufacture of the better qualities of paper is the stalk of the *Sorgo sucre*, or Chinese sugar-cane, in any of its varieties, after the juice and saccharine matter have been expressed.

In order to enable others skilled in the art to make use of my improvement in the manufacture of paper, I will proceed to describe particularly the process which I employ.

After the stalks of the Chinese sugar-cane have been passed through the crushing-rollers to extract the juice they are washed in water to rid them of the remaining saccharine and soluble matters. Where the cane is grown solely for the manufacture of paper and not for the production of molasses it may be used before it is ripe, and thus two or three crops be gathered in one season. In this case the stalks, after being crushed through rollers, are then washed to rid them of their juice and watery particles. The crushed stalks are then placed in an open vat containing a solution of caustic soda in water of the strength of about ten per cent. of caustic soda, and boiled in this solution. The object of boiling the stalks in this caustic liquor is to extract the silica, oily matters, and coloring-matter, and to open and separate the fibers, thus rendering them more susceptible to the action of the chemical with which they are subsequently treated. This boiling is continued from eight to ten hours, or until the desired separation of the fiber is produced. The stalks are then removed from the caustic liquor in which they were boiled, and washed in water until the soda is all removed. The stalks are then washed in very dilute sulphuric or muriatic acid, the water being only slightly acidulated. This effects a removal of a further portion of soluble and coloring matters. The fibrous mass

resulting from this treatment is again washed with water until free from acid, and is then immersed in a solution of chloride of lime in water of the density of from 1° to 3° of Beaumé's hydrometer. This immersion is continued for about twenty-four hours until the color of the pulp is changed from a yellowish tinge to a perfect white. The pulp is now again washed in pure water until the odor of chlorine is completely removed, and it is then washed in slightly-acidulated water of the same strength as before used, and then again with pure water until the acid is removed.

The effect of these operations is to reduce the crushed stalks to a perfectly-white homogenous mass, the knots, as well as all other parts of the cane, being completely converted into white pulp, and reduced to the condition of what is technically called "half-stuff," having entirely lost all form and structure of the cane, and being reduced to a white fibrous mass of pulp. This mass is now ready to be still further reduced by the ordinary mechanical means to an extremely fine pulp, and is then manufactured into paper in the ordinary manner.

Paper manufactured from this pulp is of a stronger texture than that made from cotton rags, the fiber resembling that of pulp made from flax, which is always employed for the best qualities of paper, and thus this article forms a perfect substitute for linen rags in the manufacture of paper, not requiring the admixture of any cotton or linen, as do straw and the other substitutes now in use, and producing a most superior quality of paper.

Another great advantage in the use of this article for the manufacture of pulp is that a much less degree of mechanical power is required, as the pulp is brought to the state of half-stuff solely by the action of the chemical agents employed in the process hereinbefore described.

The great value of this article as a substitute for linen and cotton rags in the manufacture of paper is the unlimited supply which may be obtained, while the supply of straw and other partial substitutes is so extremely limited that it is very difficult to procure a sufficient quantity to meet the demand.

What I claim as my invention, and desire to secure by Letters Patent, is—

The manufacture of pulp from the stalks of the *Sorgo sucre*, or Chinese sugar-cane, as a substitute for linen and cotton rags in the manufacture of white or the better qualities of paper, in the manner substantially as hereinabove described.

In testimony whereof I have hereunto set my hand this 27th day of October, A. D. 1857.

HENRY PEMBERTON.

Witnesses:

ISAAC HUFF,  
W. BAKEWELL.